

## UNITED STATES PATENT OFFICE

2,014,717

## FLOTATION PROCESS

Charles L. Burdick, Wilmington, Del., assignor to  
 E. I. du Pont de Nemours & Company, Wilming-  
 ton, Del., a corporation of Delaware

No Drawing. Application August 16, 1933,  
 Serial No. 685,425

8 Claims. (Cl. 209—166)

This invention relates to the treatment of ores, metallurgical products, and like heterogeneous materials containing compounds of the useful or more or less valuable metals and has for its object to provide improvement in the separation of the compounds in question by flotation, and particularly by froth flotation, from the components of the materials treated.

In accordance with the present invention it has been discovered that in the flotation treatment of ores to separate the desirable constituents therefrom, liquid media containing a mixture of sulfides, mercaptans, disulfides, polysulfides, mercaptals, thionals and equivalent derivatives of the mixture of oxygenated organic compounds obtained from the catalytic hydrogenation of carbon oxides under elevated temperatures and pressures are effective in separating the gangue from the ore according to the well known principles of froth flotation. In this process the action of the mixture of sulfides and equivalent compounds may be either to concentrate the mineral in the froth or foam and to separate the mineral from the gangue, or the action may be to concentrate the desired mineral in the form of a dispersed gangue from which the other matter is separated.

An object of the present invention is to provide new and improved frothing agents. Another object of the present invention is to provide a frothing agent which will develop a brittle and impermanent froth of sufficient buoyancy to float the mineral particles and yet of such an impermanent nature that upon removal from the activating apparatus it rapidly and completely collapses, thus affording easy separation of the mineral particles therefrom. A still further object of the invention comprises a process for the froth flotation of minerals involving the use of the mixture of the sulfides, mercaptans, the disulfides, polysulfides, and mercaptals of the higher boiling oxygenated organic compounds obtained from the catalytic hydrogenation of carbon oxides under elevated temperatures and pressures. Other objects and advantages will hereinafter appear.

My preferred frothing agents are derived from the following source. In the catalytic hydrogenation of carbon oxides under elevated temperatures and pressures a variety of straight and branch chained organic compounds containing oxygen are made. These organic compounds have a boiling point ranging from about 50° C. to a temperature of 250° C. and higher. Various methods have been proposed for manufacturing

these compounds, as, for example, the method described in the U. S. application of Roger Williams, now U. S. Patent 1,820,417. The portions of the mixture of oxygenated organic compounds obtained by Williams and equivalent processes, from which portions I generally prefer to prepare my flotation agents, are those boiling from a temperature of approximately 90° C. up. This portion boiling from 90° C. up has been fractionated systematically into a series of fractions, namely, 100—130; 130—147; 147—157; 157—195; 195—240; and 240° up. My flotation agents are made from these fractions or any other desired fraction or mixture thereof, each of which contains a plurality of organic compounds.

My flotation agents may be obtained, for example, by reacting any of the above fractions with a sulfonating agent and then with an alkali sulfide or alkali hydrogen sulfide as disclosed in the copending application of D. J. Loder, Ser. No. 685,418.

For example, the particular fraction or mixture of fractions is reacted with a strong sulfating agent such as sulfuric acid of from 96—100% strength, fuming sulfuric acid, chlorsulfuric acid, sulfur trioxide, and the like. The resulting ester is neutralized with alkali or alkaline earth caustic and the alkali salts then reacted with sodium sulfide or an equivalent alkali or alkaline earth sulfide to give the sulfide and mercaptan of the higher oxygenated organic compounds, or with a sodium hydrogen sulfide to give almost exclusively the mercaptans of these compounds. Due, of course, to the heterogeneous character of the higher oxygenated organic compounds the resulting product consists of a mixture of many different sulfides and mercaptans of the compounds present in the mixture treated. The disulfides are obtained by oxidizing the sodium salt of the mercaptan with iodine or sulfuryl chloride and the mercaptals by reacting the mercaptan with an aldehyde as described in the aforesaid application.

While it is an object of the present invention to treat ores generally in the presence of my flotation agents, the process is applicable with particular efficiency to the treatment of non-sulfide bearing ores, for example, phosphate rock, limestone, phosphite, pyrites, zircon, and ilmenite.

The quantity of my flotation agents which may be used for the treatment of a given gangue may vary within wide limits. Ordinarily, the amount used will be in the order of 1—100 parts or more to one million parts of water.

5

15

20

65

30

35

40

45

50

55

The novel flotation agents described herein may be used as the sole flotation agents or may be used in combination with flotation agents already known to the art, for example, pine oil, 5 cresylic acid, xanthate, crude oil, and the like.

The fraction or mixture of fractions of oxygenated organic compounds which are treated to obtain my flotation agent will to a certain degree determine the extent of the utility and 10 the efficiency of the compounds obtained in the flotation of a given ore. By the selection of a given fraction or a mixture of fractions it is possible, therefore, to obtain flotation agents having varying degrees of chemical and physical 15 properties with corresponding variation in flotation ability. The expert in this art, from this group of flotation agents, may then select those which are most efficient for application to his particular separation problem.

20 Any improvement to the process or products disclosed in the present specification will come within the scope of the invention without sacrificing any of the advantages that may be derived therefrom.

25 I claim:

1. In the froth flotation process of treating ores, the step which comprises utilizing as a flotation agent the mixture of oxygenated organic compounds obtained by the catalytic hydrogenation of carbon oxides under elevated temperatures and pressures converted to sulphide and mercaptan.

2. In the froth flotation process of treating ores, the step which comprises utilizing as a flotation agent the mixture of the oxygenated organic compounds obtained by the catalytic hydrogenation of carbon oxides under elevated temperatures and pressures converted to a derivative of a mixture of sulphides and mercaptans.

3. In the froth flotation process of treating ores, the step which comprises utilizing as a flotation agent the mixture of the oxygenated organic compounds obtained by the catalytic

hydrogenation of carbon oxides under elevated temperatures and pressures, which has been converted into a sulfide derivative.

4. In the froth flotation process of treating ores, the step which comprises utilizing as a 5 flotation agent the mixture of the oxygenated organic compounds obtained by the catalytic hydrogenation of carbon oxides under elevated temperatures and pressures, which has been converted into a mixture of sulfides.

5. In the froth flotation process of treating ores, the step which comprises utilizing as a flotation agent the mixture of the oxygenated organic compounds obtained by the catalytic hydrogenation of carbon oxides under elevated 15 temperatures and pressures, boiling between 130° C. and 240° C., which has been converted into a mixture of sulfides.

6. In the froth flotation process of treating ores, the step which comprises utilizing as a flotation agent the mixture of the oxygenated organic compounds obtained by the catalytic hydrogenation of carbon oxides under elevated 20 temperatures and pressures, boiling between 130° C. and 147° C., which has been converted 25 into a mixture of sulfides.

7. In the froth flotation process of treating ores, the step which comprises utilizing as a flotation agent the mixture of the oxygenated organic compounds obtained by the catalytic 30 hydrogenation of carbon oxides under elevated temperatures and pressures, boiling between 157° C. and 195° C., which has been converted into a mixture of sulfides.

8. In the froth flotation process of treating 35 ores, the step which comprises utilizing as a flotation agent the mixture of the oxygenated organic compounds obtained by the catalytic hydrogenation of carbon oxides under elevated temperatures and pressures, boiling between 40 240° C. and up, which has been converted into a mixture of sulfides.

CHARLES L. BURDICK.